

## UNITED STATES PATENT OFFICE.

GUSTAV A. REINHARDT, OF YOUNGSTOWN, OHIO.

## MOLD FOR CENTRIFUGAL CASTINGS.

No Drawing.

Application filed February 28, 1925. Serial No. 12,450.

The present invention relates to molds and more particularly to molds for use in the manufacture of iron and steel castings by the centrifugal process.

5 In this process of manufacturing castings liquid metal is poured into a mold while it revolves at high speed. Hence, a mold employed for this purpose must be highly heat resistant in addition to having the required 10 tensile strength. It is customary to make molds for centrifugal casting of a chrome-nickel steel. One method employed for the manufacture of a mold of this character is to rough forge a large ingot into the shape 15 of a round bloom. This bloom is then bored by means of a hollow drill, producing a hollow cylinder with a machined interior. This cylinder is then subjected to the necessary heat treatments to complete the mold.

20 I have discovered that a superior mold for centrifugal casting can be made from a manganese steel alloy containing preferably not less than 13% manganese to which some nickel may be added, preferably not less than 3%.

25 This percentage of manganese is sufficient to render the steel austenitic. Austenitic steel is more heat resistant and wears better than non-austenitic steel and, therefore, is particularly adaptable for the use herein specified. 30 The addition of the nickel reduces the liability of the molds made from this alloy cracking under the rapid changes in temperature to which they are subjected in use.

In carrying out my invention I may employ 25 any suitable method for making a mold from the alloy, but I prefer to cast it by the centrifugal method and then to finish it by rolling it into the shape of a seamless tube by means of any of the now existing methods, such as 40 the Pilger, automatic or similar processes for rolling seamless tubes. Austenitic steels, of which the alloy herein specified is one, usually can not be readily machined. I have found, however, that this rolling method is particu-

larly adapted for finishing and shaping an austenitic steel.

While the mold of the present invention is particularly adapted for centrifugal casting because of its high heat resistance and its superior wearing qualities, its use is not limited in this respect as it may be employed for other similar uses where these characteristics are desirable.

I claim:

1. A mold for use in the manufacture of 55 centrifugal castings of iron and steel or other metals having high melting points, consisting substantially of austenitic manganese steel, substantially as described.

2. A mold for use in the manufacture of 60 centrifugal castings of iron and steel or other metals having high melting points, consisting substantially of manganese steel containing at least 13% manganese, substantially as described.

3. A mold for use in the manufacture of 65 centrifugal castings of iron and steel or other metals having high melting points, consisting substantially of austenitic manganese steel containing a relatively small quantity of 70 nickel the minimum proportion of manganese exceeding the minimum proportion of nickel, substantially as described.

4. A mold for use in the manufacture of 75 centrifugal castings of iron and steel or other metals having high melting points, consisting substantially of austenitic manganese steel containing a relatively small amount of nickel, substantially as described.

5. A mold for use in the manufacture of 80 centrifugal castings of iron and steel or other metals having high melting points, consisting substantially of manganese steel containing at least 13% manganese and at least 3% nickel, substantially as described.

In testimony whereof I have hereunto set my hand.

GUSTAV A. REINHARDT.